

1

2,942,968

## METHOD OF SEPARATING URANIUM FROM ALLOYS

Premo Chiotti and Howard E. Shoemaker, Ames, Iowa, assignors to the United States of America as represented by the United States Atomic Energy Commission

No Drawing. Filed Nov. 15, 1957, Ser. No. 696,889

10 Claims. (Cl. 75—84.1)

This invention deals with the recovery of uranium from metallic uranium-thorium mixtures and in particular from mixtures or alloys containing the uranium in comparatively small amounts.

A number of reactors, the so-called breeder reactors, use thorium as breeding material, often in the form of a blanket arranged around the fissionable fuel material. The breeding material captures and reacts with neutrons not captured by the fissionable material and forms  $U^{233}$ , a fissionable uranium isotope, by  $n, \gamma$  reaction and subsequent  $\beta$ -decay. Such reactors using thorium as blanket material are described, for instance, in application Serial No. 721,108 on "Fast Neutron Reaction System," filed by Walter H. Zinn on January 9, 1947.

Operation of these reactors is usually discontinued at a point when the  $U^{233}$ -content is below 1 percent by weight of the neutron-reacted thorium mass. (Throughout the application percentages given are percent by weight.) On account of this small ratio of  $U^{233}$ , it is rather difficult to isolate and recover this uranium isotope. Aqueous methods using a solution of the irradiated metal have been used heretofore for this purpose, but these methods have the disadvantage that the uranium compounds obtained from these aqueous solutions have to be converted to the metal for most reactors in which the  $U^{233}$  is to be used.

It is an object of this invention to provide a process of separating uranium from thorium admixed therewith in which the uranium is recovered directly in metallic form.

It is also an object of this invention to provide a process of recovering uranium from thorium-uranium mixtures and alloys in highly pure form.

It was found that uranium is very little soluble in a magnesium-rich magnesium-thorium alloy and even less soluble in pure magnesium. It was also found that, conversely, thorium is only slightly soluble in uranium.

The various solubilities of uranium in pure magnesium and in three magnesium-thorium alloys containing 45, 35 and 16 percent of thorium, respectively, were determined. In these tests uranium was always present in an excess amount in order to make sure that the magnesium-rich phases were saturated in uranium. Various devices were used for this purpose, one being, for instance, a tantalum crucible into which the components were introduced and held under an atmosphere of argon gas. The crucible was sealed by welding, and the sealed crucible was enclosed in a welded jacket of stainless steel; the assembly was then heated in an oscillating resistance furnace which was rotated back and forth through an arc of about  $180^\circ$  C. once about every 50 seconds. For solubility determinations up to  $800^\circ$  C., rotation was carried out for 2 hours, while for those at temperatures between  $800$  and  $1200^\circ$  C. rotating times were reduced to from 15 to 10 minutes. The content of the crucible was then allowed to settle for phase separation for about the same time as rotation had been carried out and then either quenched or permitted to furnace-cool;

2

it usually took about 4 hours to furnace-cool below the melting temperature of the thorium-magnesium eutectic ( $585^\circ$  C.).

The cooled content of the crucible, which usually was a solid piece of metal containing two distinct phases was machined off in a lathe, and the central portion of each phase was removed and cleaned. Samples of both phases were analyzed, for uranium by an ammonium thiocyanate spectrophotometric method and for thorium gravimetrically by oxalate precipitation. The results of these determinations at various temperatures are compiled in Table I.

Table I

| Temp., $^\circ$ C. | Uranium Dissolved,<br>Percent $\times 10^4$ , in— |              |         |
|--------------------|---------------------------------------------------|--------------|---------|
|                    | Mg—36%<br>Th                                      | Mg—16%<br>Th | Pure Mg |
| 585                | 40                                                | 40           | 20      |
| 650                | 70                                                | 80           | 70      |
| 700                | 110                                               | 150          | 140     |
| 750                | 160                                               | 230          | 230     |
| 800                | 240                                               | 330          | 340     |
| 850                | 340                                               | 460          | 490     |
| 900                | 610                                               | 610          | 650     |
| 950                | 790                                               | 780          | 870     |
| 1,000              | 1,010                                             | 980          | 1,140   |
| 1,050              | 1,270                                             | 1,230        | 1,450   |
| 1,100              | 1,440                                             | 1,380        | 1,670   |
| 1,132              |                                                   |              |         |

These data show that the separation of uranium from thorium is better with increasing magnesium content and with decreasing temperature.

The uranium-rich phases formed in these experiments, when about 65 percent magnesium were added to the thorium mass, showed an average thorium content of  $0.9 \pm 3$  percent, the content being somewhat lower when the thorium content was lower in the magnesium-rich phase. The balance of the uranium-rich phase was essentially uranium.

It was also found that two liquid phases can be obtained at a temperature lower than the melting point of uranium by incorporating a further component, namely chromium, into the alloy. The quantity of the chromium should be high enough to form the uranium-chromium eutectic, which contains 5.2 percent of chromium, with all of the uranium present. By adding this amount of chromium, the temperature at which two liquid phases are obtained is reduced to about  $860^\circ$  C., as compared with  $1132^\circ$  C. for pure uranium. The addition of about 5 percent of chromium, based on the total uranium content present in the alloy or metallic mixture, results in the formation of a uranium-rich liquid phase containing from 0.2 to 0.6 percent of thorium when equilibrated with a magnesium-thorium alloy containing from 65 to 75 percent of magnesium. While the addition of chromium has the great advantage of a lower separation temperature, it has the disadvantage of requiring an additional step, namely, that of uranium-chromium separation if chromium-free uranium is desired. This separation can be carried out by any process known in the art; it does not form part of this invention.

The process of this invention for the separation of uranium from thorium contained in a metallic mass (the term mass is to comprise metallic mixtures and alloys) thus comprises adding magnesium to the mass in a quantity to obtain a content of from 48 to 85 percent by weight in the mixture; melting the mixture; agitating the molten mixture; allowing the mixture to settle whereby two phases, a thorium-containing magnesium-rich phase and a uranium-rich phase are formed; and separating said two phases.

The preferred magnesium content is about 58 percent, because then the magnesium-thorium eutectic is formed which requires the lowest melting temperature; the use of lower temperatures in turn results in a better uranium separation as is obvious from the uranium solubilities in Table I.

Separation of the uranium-rich phase from the magnesium-thorium alloy can be carried out either by heating the mixture to about 1150° C. when both phases are in the liquid state and the uranium-rich phase settles at the bottom, then cooling to below 585° C., preferably to room temperature, whereby the uranium-rich phase and the magnesium-thorium alloy solidify and finally separating the uranium from the alloy by mechanical means. Under these conditions the uranium-rich phase is obtained in one solid piece.

Or else, and this is the preferred method, the separation is carried out in two stages, namely, a preseparation and a final separation. Preseparation is effected by maintaining the reaction mass at a temperature above the melting point of the magnesium-thorium alloy but below the melting point of uranium, suitably just about above 585° C. in the case of the magnesium-thorium eutectic, and decanting the bulk of the liquid magnesium-thorium alloy away from a residue comprising the solid uranium-rich particles and the remainder of the magnesium-thorium alloy; recovery of the uranium from the residue is then carried out according to the methods given below. In the case of using a preseparation step less uranium is lost with the magnesium-thorium alloy on account of the lower temperature used and the lower uranium solubility at lower temperatures.

The residue, according to this invention, can be processed by two methods. One method comprises cooling of the residue to below the melting point of the magnesium-thorium alloy preferably to room temperature for solidification and separation of the solid uranium-rich phase from the solid remainder of magnesium-thorium alloy by mechanical means. According to the

other method, the residue which then has a temperature of about 585° C. is heated to above the melting point of uranium, which is about 1132° C., preferably to about 1150° C., whereby the heavy liquid uranium-rich phase, which contains less than one percent of thorium, separates and settles at the bottom of the container; the masses are then cooled to room temperature. In this case the use of the high temperature for melting the uranium does not involve a considerable uranium loss because the bulk of the magnesium-thorium alloy has been removed so that there is very little of the magnesium-thorium alloy left for dissolving uranium. The solid one-piece uranium phase is then separated from the solid one-piece magnesium-thorium alloy by mechanical means.

If chromium is added, it is preferably incorporated to the residue, that is, after the bulk of the magnesium-thorium alloy has been removed by decanting. The quantity of chromium is preferably 5.2 percent by weight based on the total amount of uranium present. The mass is then heated to a temperature within the range from 860 to 900° C., whereby the uranium-chromium eutectic settles at the bottom while the magnesium-thorium alloy collects above it. Cooling to room temperature and separation by mechanical means complete the separation.

Separation by mechanical means can either be carried out by hitting the metallic mass with a hammer whereby the two solid pieces fall apart, or by removing the magnesium-thorium alloy by lathing; the latter is preferred when there is very little magnesium-thorium alloy present with the uranium-rich phase. For further cleaning the uranium piece can be immersed in dilute nitric acid whereby any magnesium-thorium alloy still adhering to the surface is dissolved.

The thorium content of the uranium phase, which is always less than one percent, can then be reduced further by repeating the process with pure magnesium whereby the thorium is dissolved in the magnesium but very little uranium is taken up.

Table II

| Typical charge, grams | Mixing Conditions |       | Settling Conditions |         | Average chemical analyses  |                           |
|-----------------------|-------------------|-------|---------------------|---------|----------------------------|---------------------------|
|                       | Time, mins.       | ° C.  | Time, mins.         | ° C.    | Mg-rich phase, wt. percent | U-rich phase, wt. percent |
| U-1.3 a               |                   |       |                     |         |                            |                           |
| Th-26.0               | 60-120            | 1,000 | 60-120              | b 800   | {Th-35.0<br>(U-0.006       |                           |
| Mg-46.0               |                   |       |                     |         |                            |                           |
| (Th-2.25% U) e        |                   |       |                     |         |                            |                           |
| 24.0                  | 60-120            | 1,000 | 120-180             | b 800   | {Th-34.3<br>(U-0.009       |                           |
| Mg-44.0               |                   |       |                     |         |                            |                           |
| (Th-2.0% U) e         | 60-240            | 1,000 | 60-240              | d 1,000 | {Th-34.0<br>(U-0.10        |                           |
| Mg-22.0               |                   |       |                     |         |                            |                           |
| Mg-40.0               |                   |       |                     |         |                            |                           |
| (Th-53.5% U) e        | 90                | 1,000 | 10                  | d 1,200 | {Th-32.0<br>(U-0.20        | Th-1.2                    |
| Mg-43.0               | 10                | 1,200 |                     |         |                            |                           |
| U-126.7               | 10                | 1,200 | 10                  | b 1,200 | Th-32.0                    | Th-0.85                   |
| Th-10.3               |                   |       |                     |         |                            |                           |
| Mg-19.5               |                   |       |                     |         |                            |                           |
| U-145.5               | 15                | 1,200 | 15                  | d 1,200 | Th-34.0                    | Th-0.68                   |
| Th-10.5               |                   |       |                     |         |                            |                           |
| Mg-19.6               |                   |       |                     |         |                            |                           |
| (Th-53.5% U) e        | 44.7              | 1,200 | 10                  | b 1,200 | Th-34.0                    | Th-0.84                   |
| Mg-41.7               |                   |       |                     |         |                            |                           |
| U-158.1               | 15                | 1,200 | 10                  | b 1,200 | Th-3.0                     | Th-0.3                    |
| Th-1.1                |                   |       |                     |         |                            |                           |
| Mg-19.7               |                   |       |                     |         |                            |                           |
| (U-5.5% Cr) e         | 44.7              | 900   | 60-120              | d 900   | {Th-30<br>(U-0.053         | Th-0.4                    |
| Th-15.2               |                   |       |                     |         |                            |                           |
| Mg-43.7               |                   |       |                     |         |                            |                           |
| (U-5.5% Cr) e         | 178.5             | 900   | 60                  | d 900   | {Th-3.6<br>(U-0.052        | Th-0.2                    |
| Th-1.0                |                   |       |                     |         |                            |                           |
| Mg-19.0               |                   |       |                     |         |                            |                           |

a Uranium shavings.

b Sample furnace-cooled from temperature indicated.

c Arc-melted alloy.

d Sample quenched instead of furnace-cooled, from temperature indicated.

In view of the high reactivity of the metals involved, it is advisable to carry out the separation process under the exclusion of air; this is best accomplished by operating in an inert atmosphere of helium or argon gas.

The magnesium-rich phase can be processed by distillation for the separation of the magnesium from the thorium.

A number of uranium-thorium separations were carried out using a technique similar to that employed for the determination of the solubilities and described above. The conditions and results together with the compositions of the mixtures melted are compiled in Table II.

The balance of the magnesium-rich phase in each of the above examples was magnesium and that of the uranium-rich phase uranium. The experiments show that a good separation is accomplished by the process of this invention.

It will be understood that this invention is not to be limited to the details given herein, but that it may be modified within the scope of the appended claims.

What is claimed is:

1. A process of recovering uranium from metallic uranium-thorium mixtures, comprising adding magnesium to the mass in a quantity to obtain a content of from 48 to 85 percent by weight; melting and forming a magnesium-thorium alloy at a temperature of between 585 and 800° C.; agitating the mixture; allowing the mixture to settle whereby two phases, a thorium-containing magnesium-rich liquid phase and a solid uranium-rich phase are formed; and separating said two phases.

2. The process of claim 1 wherein the phases are separated by heating to about 1150° C. whereby both phases are melted and the uranium-rich phase settles at the bottom, then cooling both phases to room temperature for solidification, and separating the uranium-rich phase from the magnesium-thorium phase by mechanical means.

3. The process of claim 1 wherein a phase preseparation is first carried out by heating the phases to above the melting point of the magnesium-thorium alloy, but below the melting point of the uranium and decanting the bulk of the magnesium-thorium alloy away from a residue containing the remainder of the magnesium-thorium alloy and solid particles of the uranium-rich phase.

4. The process of claim 3 wherein magnesium is added

in a quantity of about 58 percent and the preseparation temperature is about 585° C.

5. The process of claim 3 wherein said residue is cooled to room temperature whereby the uranium-rich phase and the remainder of the magnesium-thorium alloy solidify and the phase is separated from the remainder by mechanical means.

6. The process of claim 3 wherein said residue is heated to about 1150° C. until the uranium-rich phase is melted and has settled at the bottom, it is then cooled to room temperature and the uranium-rich phase is separated from said remainder of the alloy by mechanical means.

7. The process of claim 3 wherein from 5 to 5.2 percent of chromium, based on the quantity of uranium, is added to the residue, the mixture thus obtained is heated to from 860 to 900° C. until a liquid light magnesium-thorium alloy has separated from a liquid heavy uranium-chromium eutectic, the alloy and the eutectic are then cooled to room temperature and separated by mechanical means.

8. The process of claim 1 wherein melting is carried out in an inert atmosphere.

9. The process of claim 1 wherein magnesium is added to the separated uranium-rich phase whereby a further decontamination from any thorium still present with the uranium is obtained.

10. A process of recovering uranium from metallic uranium-thorium mixtures, comprising adding magnesium in a quantity to obtain a content of about 58 percent in the mixture and about 5.2 percent of chromium based on the uranium present in the mass; heating the mixture to about 900° C. and agitating it for thorough contacting; allowing the mixture to settle whereby two phases, a thorium-containing magnesium-rich phase and a uranium-chromium eutectic phase are formed; and separating said two phases.

#### References Cited in the file of this patent

Lawroski: "Survey of Separation Processes," P/823, International Conference on the Peaceful Uses of Atomic Energy, vol. 9, pages 580-582 (1956).

Finniston et al.: "Metallurgy and Fuels," Progress in Nuclear Energy, vol. 5, McGraw-Hill Book Co., N.Y. (1956), pages 169, 212, 253.